

## UNITED STATES PATENT OFFICE

EDWARD R. WILLIAMS, OF LATROBE, PENNSYLVANIA, ASSIGNOR TO VULCAN MOLD AND IRON COMPANY, OF LATROBE, PENNSYLVANIA, A CORPORATION OF PENNSYLVANIA

## INGOT MOLD

No. Drawing. Application filed June 22, 1929. Serial No. 373,058.

Iron ingot molds made by the direct metal process or with iron as it comes in the molten state from the blast furnace have a number of disadvantages. The temperature of the molten iron from the time it leaves the blast furnace until it is poured into the mold becomes lower which reduces by precipitation the amount of carbon held in solution. This precipitated carbon or "kish" promotes porosity in the mold casting, particularly at its top. The temperature of the molten iron being comparatively low reduces its fluidity, and unless the mold wall is fairly thick, as four inches or more, the metal tends to "cold-shut" or solidify in layers which results in a scrap mold. It is therefore impracticable to make good ingot molds with a small wall thickness by the direct metal process.

The chemical analysis of direct metal varies greatly so that such metal cannot make molds of uniform composition. The carbon which precipitates from direct metal as graphite is in large flat flakes which promotes the growth and the consequent fire cracking of the ingot mold after its repeated heating and cooling in use. Large graphite flakes render the metal relatively weak as compared with metal having small graphite flakes.

By melting pig iron in a cupola or a similar re-melting medium better physical properties are produced than by the direct metal process. The high melting temperature prevailing in the cupola gives the metal better fluidity than the direct metal from a blast furnace has and therefore gives the casting a smoother surface. The cupola method of producing cast iron affords a better control of the melting temperature than is obtainable by the direct metal method, owing to the ease of manipulating the coke ratio in a short period of time. Also the cupola method gives better control of the composition of the iron as to the percentage of silicon, phosphorus, carbon and manganese therein. Cupola metal as generally made has a serious disadvantage, particularly when cast as ingot molds of large size. During the melting operation sulphur is absorbed from the fuel to the extent of from .02% to .05%, which pro-

duces sulphur in the resultant casting of over .05% and sometimes as high as .15%, depending on conditions. High sulphur content renders the ingot molds "red-short" which, if the mold wall has insufficient structural strength, allows it to crack. Sufficient structural strength is produced only by having the mold wall thicker than is necessary to properly absorb the heat from the solidifying ingot.

I have discovered that ingot molds made of cupola iron with the sulphur under .05% are highly resistant to cracking even when they have a relatively large sectional area. The low sulphur cupola iron ingot molds therefore fail only by the normal process of growth and fire cracking.

In the preferable practice of my invention I employ a cupola in which the metal charges are melted. A suitable de-sulphurizer such as soda ash is added to the molten metal in sufficient quantity to reduce the sulphur content below .05%. The de-sulphurized molten metal is then poured into the ingot mold in the usual manner.

## I claim:

An ingot mold made of cupola cast iron which contains sulphur under .05% and has high resistance to cracking through sudden expansion.

In testimony whereof, I hereunto affix my signature.

EDWARD R. WILLIAMS.